

# United States Patent

[11] 3,625,782

[72] Inventors **Adolf E. Oberth**  
**Fair Oaks;**  
**Rolf S. Bruenner, Orangevale, both of**  
**Calif.**  
[21] Appl. No. **726,649**  
[22] Filed **May 2, 1968**  
[45] Patented **Dec. 7, 1971**  
[73] Assignee **Aerojet-General Corporation**  
**El Monte, Calif.**

3,092,526 6/1963 Philipson ..... 149/76 X  
3,172,794 3/1965 Ender ..... 149/19  
3,214,304 10/1965 Vriesen ..... 149/76 X  
3,266,959 8/1966 Ackley ..... 149/19  
3,291,660 12/1966 Oberth et al. ..... 149/19  
3,340,111 9/1967 Stammler ..... 149/19

*Primary Examiner*—Benjamin R. Padgett  
*Attorneys*—Edward O. Ansell, D. Gordon Angus and Reid  
Anderson

[54] **SOLID PROPELLANTS CONTAINING BURNING RATE DEPRESSANTS**  
12 Claims, 10 Drawing Figs.

[52] U.S. Cl. .... 149/19,  
149/20  
[51] Int. Cl. .... C06d 5/06  
[50] Field of Search. .... 149/19, 20

[56] **References Cited**

UNITED STATES PATENTS

3,024,144 3/1962 Sammons ..... 149/76 X

**ABSTRACT:** This patent described novel solid ammonium perchlorate containing propellant compositions containing powerful burning-rate depressants which are potential bases, that is, compounds which are capable of releasing free bases. The burning-rate depressants of this invention do not reduce the specific impulse of the propellant, nor do they interfere with cure reactions or adversely affect the physical properties of the cured propellant.



INVENTORS.  
 ADOLF E. OBERTH  
 ROLF S. BRUENNER  
 BY  
*lynn shay*  
 ATTORNEYS



INVENTORS.  
ADOLF E. OBERTH  
ROLF S. BRUENNER  
BY

*Lyons Lyons*  
ATTORNEYS



FIG. 5.



FIG. 6.

INVENTORS,  
ADOLF E. OBERTH  
ROLF S. BRUENNER  
BY  
*Lyon & Lyon*  
ATTORNEYS



FIG. 8.

INVENTORS  
 ADOLF E. OBERTH  
 ROLF S. BRUENNER  
 BY  
*Tyson & Tyson*  
 ATTORNEYS



FIG. 9.



FIG. 10.

INVENTORS.  
 ADOLF E. OBERTH  
 ROLF S. BRUENNER  
 BY *Lyons & Lyons*  
 ATTORNEYS

**SOLID PROPELLANTS CONTAINING BURNING RATE DEPRESSANTS**

**BACKGROUND OF THE INVENTION**

The field of the present invention pertains to novel solid rocket propellants and their preparation.

Solid rocket propellants employing ammonium perchlorate as an oxidizing agent are well known. In general, propellants based upon ammonium perchlorate have a high burning rate. In many solid rocket applications, it is desirable to have a propellant which will provide a slower burning rate than normally can be had with ammonium perchlorate propellants. Therefore, it has been proposed to use various burning-rate depressants to control and reduce the burning rate of ammonium perchlorate propellants. Typical of such known burning-rate depressants is calcium oxalate. However, it is necessary to use calcium oxalate in rather substantial quantities if the desired burning-rate suppression is to be obtained. Moreover, calcium oxalate does not contribute to the energy of the propellant and hence, when used in effective burning-rate depressing amounts, reduces the specific impulse of the propellant.

According to the present invention there has now been found potential bases which are uniquely adapted to the reduction of the burning rate of ammonium perchlorate containing propellants. These additives are substantially more effective than calcium oxalate in that they require only about one-tenth or less of the concentration of calcium oxalate in order to provide the same degree of burning-rate suppression. In addition, the burning-rate additives of the present invention do not decrease the propellant's specific impulse.

**SUMMARY OF THE INVENTION**

Briefly, the present invention comprises novel solid ammonium perchlorate containing rocket propellants containing therein potential bases which are stable under conventional solid propellant curing conditions but which yield at least some free base upon propellant combustion. The amine precursors reduce the burning rate of the propellant without adversely affecting the specific impulse or the physical properties thereof. The invention further comprises the formulation of novel propellants containing the burning-rate depressants referred to above.

The precursors are used in an effective burning rate reducing amount, normally from about 0.01 percent to about 5 percent by weight of the propellant. The optimum amount for any propellant is dependent upon the propellant formulation and performance desired.

While not bound by any theory, it is believed that the novel burning-rate depressants of the present invention act as sources of free nonvolatile bases such as amines, that is, compounds which release bases upon thermal decomposition only. It has been found that nonvolatile free organic amines in a propellant binder drastically reduce the burning rate, apparently due either to the generation of ammonia or to the prevention of the buildup of a hydrogen-perchlorate-rich surface on the  $\text{NH}_4\text{ClO}_4$  particles. However, the incorporation of strongly basic free amines in a propellant is impractical, since it was found that the ordinary binder systems used in the solid propellants will not satisfactorily cure in their presence. The precursor compounds of the present invention are believed to generate the free nonvolatile amines in situ, and therefore permit the curing of the propellant and at the same time yield, upon decomposition, the free nonvolatile amines which suppress the buildup of perchloric-acid-rich surfaces on the  $\text{NH}_4\text{ClO}_4$  particles.

The control of the ammonia generation and perchloric acid buildup is believed to be significant for the following reasons. It is well known that in an ammonia atmosphere, the decomposition of ammonium perchlorate is considerably slowed down. It is believed that the decomposition of ammonium perchlorate is preceded by a dissociation into ammonia and hydrogen perchlorate, followed by desorption where am-

monia, because of its lower molecular weight, diffuses away faster, leaving a hydrogen-perchlorate-rich surface. In the present invention, it is believed that the burning-rate depressants of this invention prevent temporarily the buildup of a hydrogen-perchlorate-rich surface. The compounds of the present invention are very beneficial in controlling the burning rate of ammonium perchlorate propellants. In addition, the compounds of the present invention are fully compatible with the binder system and do not interfere with curing. These compounds are also sufficiently soluble in the binder to allow themselves to be adsorbed onto the ammonium perchlorate.

Accordingly, it is an object of the present invention to provide a novel class of solid rocket propellants.

More particularly, it is an object of the present invention to provide a novel class of solid rocket propellants having a decreased burning rate and containing precursors of free organic amines.

Yet another object of the present invention is to provide the means for controlling the burning rate of ammonium perchlorate propellants without adversely affecting the specific impulse.

Still another object of the present invention is the provision of burning-rate modifier compounds which are effective in ammonium perchlorate propellants and do not interfere with the cure system or the physical properties of the cured propellant.

These and other objects and advantages of the present invention will become apparent from the detailed description which follows.

**DESCRIPTION OF THE PREFERRED EMBODIMENTS**

New classes of burning-rate modifiers within the scope of the present invention are those compounds derived from amines which will yield free amines upon thermal decomposition or those which are capable of exchanging the amine constituent. The present invention is not limited to amine derivatives, however, but extends to compounds which are potential bases, that is, compounds or compositions which, at elevated temperatures, are converted into or release free bases and are readily adsorbed or coated onto the oxidizer (ammonium perchlorate or other ammonium salts with an oxidizing anion like  $\text{NO}_3^-$  included are also salts of ammonium derivatives, such as hydroxyl-ammonium).

The amine derivatives within the scope of the present invention include ammonium salts of organic amines having the formula:



wherein  $\text{R}_1$  and  $\text{R}_2$  are either alkyl groups or hydrogen, and  $\text{R}_3$  is preferably a hydrocarbon chain containing from eight to 30 carbon atoms. Any of the R-groups may contain one or more functional groups such as hydroxyl, etc. Examples of acid used to prepare the salts from the above amines include hydrochloric, sulfuric, nitric, perchloric, hydrogen borofluoride and perfluoroacetic.

The invention also includes quaternary ammonium salts having the formula:



wherein  $\text{R}_4$ ,  $\text{R}_5$ ,  $\text{R}_6$  and  $\text{R}_7$  are alkyl groups, preferably where at least one R group is a hydrocarbon chain containing from about eight to about 30 carbon atoms. Any of the R-groups may contain one or more functional groups such as hydroxyl,

carboxyl, etc. X is any of the stable inorganic or organic anions, i.e., chloride, nitrate, sulfate, phosphate, etc. Included are also quaternary ammonium salts which are derived from oligo- and polyamines.

An example of the preparation of quaternary ammonium salts (1936) trimethylhexadecylammonium iodide wherein 13.5 g. dimethylhexadecylamine are dissolved in approximately 100 ml. methylethylketone (MEK) and then 7 g. methyl iodide added under stirring. This mixture is heated to the boiling point of MEK and isopropanol is added until all of the precipitated quaternary ammonium salt has dissolved. The clear solution is allowed to cool to room temperature whereupon the salt crystallizes out. After washing with MEK the compound was dried under vacuum. White crystalline solid, melting point close to that reported in the literature (247° C.) (Macroski, Bulletin de la Societe Chimique de France (5) 3 (1936) 500); yield is nearly quantitative.

Another example of the preparation of quaternary ammonium salts is trimethyldodecylammonium toluenesulfonate wherein 10 g. dimethyldodecylamine are dissolved in about 50 ml. methylethylketone and 9.3 g. methyl p-toluenesulfonate added under stirring. The quaternary ammonium salt starts to crystallize out already at room temperature. To complete the reaction the solution is heated to the b.p. of MEK and just enough isopropanol added to completely dissolve any precipitate. The desired compound crystallizes out on cooling to room temperature. It is filtered off, washed with MEK and dried under vacuum. White, crystalline solid; yield nearly quantitative.

A still further example of the preparation of quaternary ammonium salts is trimethyldodecylammonium metaphosphate wherein a cold solution of 1.2 g. water-soluble sodium metaphosphate in 100 ml. water, a hot solution of 4 g. trimethyldodecylammonium toluenesulfonate in about 30 ml.

water is added under rapid stirring, whereupon the quaternary ammonium metaphosphate precipitates immediately. It is filtered off, washed with plenty of cold water and dried under vacuum. White solid, soluble inorganic solvents like  $\text{CHCl}_3$  and others.

The following quaternary ammonium halide compounds have also been found to be useful in this invention.

| Iodides (X=I) |  | R <sub>1</sub>               | R <sub>2</sub>               | R <sub>3</sub> | R <sub>4</sub> |
|---------------|--|------------------------------|------------------------------|----------------|----------------|
| Compound No.  |  |                              |                              |                |                |
| 1             |  | $\text{C}_{12}\text{H}_{25}$ | $\text{CH}_3$                | $\text{CH}_3$  | $\text{CH}_3$  |
| 2             |  | $\text{C}_{10}\text{H}_{23}$ | $\text{CH}_3$                | $\text{CH}_3$  | $\text{CH}_3$  |
| 3             |  | $\text{C}_{10}\text{H}_{23}$ | $\text{C}_{10}\text{H}_{23}$ | $\text{CH}_3$  | $\text{CH}_3$  |

  

| Bromides (X=Br) |  | R <sub>1</sub>               | R <sub>2</sub>               | R <sub>3</sub>               | R <sub>4</sub> |
|-----------------|--|------------------------------|------------------------------|------------------------------|----------------|
| Compound No.    |  |                              |                              |                              |                |
| 1               |  | $\text{C}_{10}\text{H}_{23}$ | $\text{C}_6\text{H}_{11}$    | $\text{CH}_3$                | $\text{CH}_3$  |
| 2               |  | $\text{C}_{10}\text{H}_{23}$ | $\text{C}_{10}\text{H}_{23}$ | $\text{CH}_3$                | $\text{CH}_3$  |
| 3               |  | $\text{C}_{10}\text{H}_{23}$ | $\text{C}_{10}\text{H}_{23}$ | $\text{C}_{10}\text{H}_{23}$ | $\text{CH}_3$  |

  

| Chlorides (X=Cl) |  | R <sub>1</sub>               | R <sub>2</sub>               | R <sub>3</sub> | R <sub>4</sub> |
|------------------|--|------------------------------|------------------------------|----------------|----------------|
| Compound No.     |  |                              |                              |                |                |
| 1                |  | $\text{C}_{10}\text{H}_{23}$ | $\text{CH}_3$                | $\text{CH}_3$  | $\text{CH}_3$  |
| 2                |  | $\text{C}_{10}\text{H}_{23}$ | $\text{CH}_3$                | $\text{CH}_3$  | $\text{CH}_3$  |
| 3                |  | $\text{C}_{10}\text{H}_{23}$ | $\text{CH}_3$                | $\text{CH}_3$  | $\text{CH}_3$  |
| 4                |  | $\text{C}_{10}\text{H}_{23}$ | $\text{C}_6\text{H}_{11}$    | $\text{CH}_3$  | $\text{CH}_3$  |
| 5                |  | $\text{C}_{10}\text{H}_{23}$ | $\text{C}_{10}\text{H}_{23}$ | $\text{CH}_3$  | $\text{CH}_3$  |

Other quaternary ammonium salts useful in this invention and containing hydroxyl groups include:

|          | R <sub>1</sub>                                  | R <sub>2</sub>                                  | R <sub>3</sub>                     | R <sub>4</sub>                                  | X                         |
|----------|-------------------------------------------------|-------------------------------------------------|------------------------------------|-------------------------------------------------|---------------------------|
| (a)..... | $\text{CH}_3\text{CH}_2\text{OH}$               | $\text{CH}_2\text{CH}_2\text{OH}$               | $-\text{CH}_2\text{CH}_2\text{OH}$ | $-\text{CH}_3$                                  | I                         |
| (b)..... | Same as above.....                              | Same as above.....                              | $-\text{CH}_3$                     | $-\text{CH}_3$                                  | I                         |
| (c)..... | $\text{CH}_2-\text{CH}(\text{OH})-\text{CH}_3$  | $-\text{CH}_2-\text{CH}(\text{OH})-\text{CH}_3$ | $\text{C}_{10}\text{H}_{23}$       | $-\text{CH}_3$                                  | $\text{O}_2\text{SOCH}_3$ |
| (d)..... | $-\text{CH}_2-\text{CH}(\text{OH})-\text{CH}_3$ | $-\text{C}_{10}\text{H}_{23}$                   | $-\text{CH}_3$                     | $-\text{CH}_3$                                  | Cl                        |
| (e)..... | Same as above.....                              | $-\text{CH}_2\text{CH}_2\text{OH}$              | $-\text{CH}_2\text{CH}_2\text{OH}$ | $-\text{C}_{10}\text{H}_{23}$                   | Cl                        |
| (f)..... | $-\text{CH}_3\text{CH}_2\text{OH}$              | do.....                                         | $-\text{C}_{10}\text{H}_{23}$      | $-\text{CH}_3$                                  | Cl                        |
| (g)..... | Same as above.....                              | do.....                                         | $-\text{C}_{10}\text{H}_{23}$      | $-\text{CH}_3$                                  | Cl                        |
| (h)..... | do.....                                         | do.....                                         | Same as above.....                 | $-\text{C}_{10}\text{H}_{23}$                   | Br                        |
| (i)..... | $-\text{CH}_2-\text{CH}(\text{OH})-\text{CH}_3$ | $-\text{CH}_2-\text{CH}(\text{OH})-\text{CH}_3$ | do.....                            | $-\text{CH}_3$                                  | $\text{O}_2\text{SOCH}_3$ |
| (j)..... | $-\text{CH}_2-\text{CH}(\text{OH})-\text{CH}_3$ | $-\text{CH}_2-\text{CH}_2\text{OH}$             | $-\text{CH}_2\text{CH}_2\text{OH}$ | $-\text{C}_{10}\text{H}_{23}$                   | Cl                        |
| (k)..... | Same as above.....                              | $-\text{C}_{10}\text{H}_{23}$                   | $-\text{CH}_3$                     | $-\text{CH}_3$                                  | Cl                        |
| (l)..... | $-\text{CH}_2\text{CH}_2\text{OH}$              | $-\text{CH}_2\text{CH}_2\text{OH}$              | $-\text{CH}_3$                     | $-\text{CH}_3$                                  | I                         |
| (m)..... | Same as above.....                              | do.....                                         | $\text{CH}_2\text{CH}_2\text{OH}$  | $-\text{CH}_3$                                  | I                         |
| (n)..... | $-\text{C}_{10}\text{H}_{23}$                   | $-\text{C}_2\text{H}_5$                         | $-\text{CH}_3$                     | $-\text{CH}_3$                                  |                           |
| (o)..... | Same as above.....                              | $-\text{CH}_3$                                  | $-\text{CH}_3$                     | $-\text{CH}_3$                                  | Same as above.            |
| (p)..... | do.....                                         | $-\text{CH}_3$                                  | $-\text{CH}_3$                     | $-\text{CH}_3$                                  | Do.                       |
| (q)..... | $-\text{C}_{10}\text{H}_{23}$                   | $-\text{CH}_3$                                  | $-\text{CH}_2\text{CH}_2\text{OH}$ | $-\text{CH}_2\text{CH}_2\text{OH}$              | Do.                       |
| (r)..... | $-\text{CH}_3$                                  | $-\text{CH}_2\text{CH}_2\text{CN}$              | Same as above.....                 | Same as above.....                              | Do.                       |
| (s)..... | $-\text{CH}_3$                                  | $-\text{CH}_3$                                  | $-\text{CH}_3$                     | $-\text{CH}_2-\text{CH}(\text{OH})-\text{CH}_3$ | Do.                       |
| (t)..... | $-\text{CH}_3$                                  | $\text{NC}-\text{CH}_2\text{CH}_2-$             | $-\text{CH}_2\text{CH}_2\text{OH}$ | $-\text{CH}_2\text{CH}_2\text{OH}$              | Do.                       |
| (u)..... | $-\text{CH}_3$                                  | $-\text{CH}_3$                                  | $-\text{CH}_3$                     | $-\text{CH}_2\text{CH}_2\text{OH}$              | Do.                       |
| (v)..... | $-\text{CH}_3$                                  | $-\text{CH}_2-\text{CHOH}-\text{CH}_3$          | $-\text{CH}_2\text{CH}_2\text{OH}$ | $-\text{CH}_2\text{CH}_2\text{OH}$              | Do.                       |
| (w)..... | $-\text{CH}_3$                                  | $-\text{CH}_3$                                  | $-\text{CH}_2\text{CH}_2\text{OH}$ | $-\text{CH}_2\text{CH}_2\text{OH}$              | Do.                       |
| (x)..... | $-\text{CH}_3$                                  | $-\text{CH}_3$                                  | $-\text{CH}_3$                     | $-\text{CH}_2\text{CH}_2\text{OH}$              | Do.                       |
| (y)..... | $-\text{CH}_3$                                  | $-\text{C}_{10}\text{H}_{23}$                   | $-\text{CH}_2\text{CH}_2\text{OH}$ | $-\text{CH}_2\text{CH}_2\text{OH}$              | Do.                       |
| (z)..... | $-\text{CH}_3$                                  | $-\text{CH}_3$                                  | $-\text{C}_{10}\text{H}_{23}$      | $-\text{C}_{10}\text{H}_{23}$                   | Do.                       |

Polymeric quaternary ammonium salts with OH groups are also included, and are illustrated by:



Another class of burning-rate suppressors within the scope of the present invention are zwitterionic compounds, including betaines and betaine analogues having the formula:



wherein  $\text{R}_9$ ,  $\text{R}_{10}$  and  $\text{R}_{11}$  are alkyl groups;  $\text{R}_9$  is any linear or branched hydrocarbon group, normally alkylene; and  $\text{Y}$  may be any of the stable inorganic or organic groups such as  $-\text{OBF}_3$ ,  $-\text{SO}_3$  and  $-\text{COO}$ . In the above formula, the  $\text{R}_9$ -group can be omitted in which case the  $\text{Y}$ -group ( $\text{BF}_3$ , 0, etc.) is attached directly to the nitrogen. In the above formula, any of the  $\text{R}$ -groups may comprise a hydrocarbon structure from eight to 30 carbon atoms. Also, any of the  $\text{R}$ -groups may contain one or more functional groups such as hydroxyl, carboxyl, etc. Included also are structures which contain more than one functional group such as hydroxyl, carboxyl, etc. Included also are structures which contain more than one anionic  $\text{Y}$ -group.

An example for the preparation of a Betaine Analogue having the formula:



(according to T. L. Gresham et al., J.A.C.S. 73, 3,168, (1951)).

To a solution of 21.3 g. dimethyldodecylamin in 125 ml. ether and 38 ml.  $\text{H}_3\text{C}-\text{CN}$  7.2 g.  $\beta$ -propiolactone were added under stirring, whereupon a white solid formed. After standing for 16 hours, the solid was filtered off and washed with ether. The compound was dried under vacuum and kept over  $\text{P}_2\text{O}_5$ ; yield 24 g. (81 percent).

An example for the preparation of a tertiary amine- $\text{BF}_3$  adduct having the formula:



wherein 0.8 moles of dry ether were placed in a three-neck flask and  $\text{BF}_3$  was passed in through a glass-fritted tube until vapors of  $\text{BF}_3$  could be detected above the solution; some more ether was then added to convert all excess  $\text{BF}_3$  to the  $\text{BF}_3$ -etherate. To this solution 0.8 moles of dimethyl-dodecylamine were added under stirring. The ether was then removed under aspirator vacuum. After this, all remaining  $\text{BF}_3$ -etherate was distilled off under oil pump vacuum at 80° C. The residue crystallized at room temperature and was recrystallized from heptane; white flakes.

An example for the preparation of an oxyfluorobetaine having the formula:



(according to H. Meerwein et al., J. Prakt. Chem. (2) 154, 83 (1940)), wherein 0.25 moles of



and 0.25 moles of dodeceneoxide were heated under stirring in a 100° C. oil bath. At 70°-75° C. the reaction starts with an exotherm, which takes the mixture of about 115°-120° C. At the same time the color changes from a pale yellow to the color of honey. The compound is a rather viscous liquid at 90° C. and vaselinelike at room temperature.

An example for the preparation of a sulfobetaine (according to J. H. Helberger, Ann. 588, 71 (1954)) wherein 6.107 g.  $\gamma$ -propanesultone and 10.65 g. dimethyldodecylamine are heated in about 50 ml. xylene. At ~95° C. an exothermic reaction starts under precipitation of the desired compound. The mixture is taken to ca. 140° C. and held there for 10 mins. to complete the reaction. After cooling to room temperature the solvent is removed by filtering; the residue is stirred with acetone (which facilitates filtering), filtered and washed several times with acetone. The compound is then dried under vacuum at about 60°-70° C.; white solid.

Another class of compounds within the scope of the present invention are the substituted ureas having the formula:



wherein  $\text{R}_{12}$  is a hydrocarbon group, and  $\text{R}_{13}$ ,  $\text{R}_{14}$  and  $\text{R}_{15}$  are hydrogen or hydrocarbon groups, preferably with one or more of the  $\text{R}$ -groups consisting of hydrocarbon chains from about eight to about 30 carbon atoms. Any of the  $\text{R}$ -groups may contain one or more functional groups such as hydroxyl, carboxyl, etc. Also included are derivatives of biuret, guanidine and similar compounds.

The following is an example for the preparation of a substituted urea having the formula  $[(\text{CH}_2)_3-\text{NH}-\text{CO}-\text{NH}-\text{C}_{12}\text{H}_{25}]_2$ : 18.5 g. dodecylamine and 8.4 g. hexamethylene diisocyanate are dissolved separately in heptane and then the isocyanate solution is added to the amine solution with good stirring. The product precipitates out immediately. It is filtered off and washed thoroughly with heptane; white solid.

Still further, the invention includes any of the metal salts which form stable complexes with amines. The amino nitrogen can carry at least one hydrocarbon group with or without other functional or complexing groups. Preferably the hydrocarbon group contains from about eight to 30 carbon atoms. An example of such a compound is the zinc complex:



The preparation of the potential base compounds is not new, and the general methods can be found in e.g., Houben-Weyl, Methoden der organischen Chemie, Vol. XI/2, Stuttgart 50 Georg Thieme Verlag, 1958, pp. 591-613 (for quaternary ammonium compounds including betaines and betaine analogues), Vol. VIII (1952), pp. 157-158 (for substituted ureas), pp. 180-183 (for substituted guanidinium salts), Vol. I/1 (1958), pp. 391-410 (for urea clathrates). The synthesis of sulfobetaines can be found in: R. F. Fischer, Ind. & Eng. Chem. Vol. 56, No. 3, p. 44 (1964) etc.

The following examples are presented solely to illustrate the invention and should not be regarded as limiting in any way. In the examples, the parts and percentages are by weight unless otherwise indicated.

Amine precursor compounds were evaluated, by incorporation at an 0.3 percent level into a propellant consisting of 86 percent solids (76 percent ammonium perchlorate, and 10 percent powdered aluminum). The additive replaced an equivalent amount of the binder. Direct addition of the respective amine precursor compound to the binder is preferred, though in special cases the oxidizer was precoated with the material. Processing was done at 115°-125° F. The propellants were cured at 135° F. in bulk for preparation of solid strands. Since the response of a propellant towards such burning-rate modifiers depends strongly on the binder, two representative binders were used for testing.

| Binder No. 1                                    |        |  |
|-------------------------------------------------|--------|--|
| Polypropylene ether diol                        | 28.43% |  |
| Polypropylene ether triol                       | 41.10% |  |
| Isodecylglaconate                               | 25.00% |  |
| Hexamethylene diisocyanate (107 eqs/100 eqs OH) | 5.47%  |  |
| N-phenyl betanaphthylamine                      | 0.1%   |  |

Catalyst is either FeAA (0.015-0.03 percent) or dibutyltin-dilauroate (0.05 percent).

Binder No. 2

|                                              |       |
|----------------------------------------------|-------|
| Carboxy-terminated polybutadiene (100 eqs)   | 68.0% |
| Trimethylaziridine phosphine oxide (120 eqs) | 2.07% |
| Isooctylpelargonate                          | 30.0% |

The following compounds are a few examples of those synthesized and tested:

- (a) 
- (b) 
- (c) 
- (d)  $[(H_{37}C_{18}N(CH_3)_2)_2I]$
- (e)  $[(H_{37}C_{18})_2N(CH_3)_2I]$
- (f)  $[(H_{37}C_{18})_3N(CH_3)_2I]$

In the Binder No. 1 system (FIG. 1) it is seen that the (3) (f) is more effective than the iodide (3) of an identical cation. If compared with the iodide series  $[(RN(CH_3)_2)_2I]$  when  $R=(1) C_{12}H_{25}$  and (2)  $C_{18}H_{33}$  then compound (e)  $R=C_{18}H_{37}$  is the least effective, whereas (2)  $R=C_{18}H_{33}$  is the most effective. The mole concentrations of these compounds are 2.82, 2.43 and 1.48 respectively. The effectiveness passes through a maximum. The bromides (b) and (c) (FIG. 2) (Binder No. 1) compare favorably with any of the other compounds.

Sulfobetaines of the following formula were used in Binder No. 1 (FIG. 3), and Binder No. 2 (FIG. 4):



In addition to the two compounds with  $R_1=C_{12}H_{25}$  and  $R_1=C_{18}H_{33}$  and  $R_2=R_3=CH_2R_4(-CH_2-)_3$ , a compound with  $R_1=C_{18}H_{37}$  was prepared, which proved to be the most effective one in both systems (FIGS. 3 and 4).

Ureas of the formula:



WITH  $R_1$  and  $R_2$  hydrocarbon was used.

The following compounds were prepared and tested:

- a.  $\text{O}=\text{C}(\text{NH}-\text{C}_{18}\text{H}_{37})_2$   
 b.  $\text{f} (\text{CH}_2)_3-\text{NH}-\text{CO}-\text{NH}-\text{C}_{12}\text{H}_{25})_2$   
 c.  $\text{f} (\text{CH}_2)_3-\text{NH}-\text{CO}-\text{NH}-\text{C}_{18}\text{H}_{33})_2$   
 d.  $\text{f} (\text{CH}_2)_3-\text{NH}-\text{CO}-\text{NH}-\text{C}_{18}\text{H}_{37})_2$   
 e.  $\text{f} (\text{C}_{18}\text{H}_{37})-\text{NH}-\text{CO}-\text{NH}-\text{C}_{12}\text{H}_{25})_2$   
 f.  $\text{f} (\text{C}_{18}\text{H}_{37})-\text{NH}-\text{CO}-\text{NH}-\text{C}_{18}\text{H}_{37})_2$

The results are shown in FIGS. 5-8. In both systems, Binder No. 1 (FIGS. 5 and 6) and Binder No. 2 (FIGS. 7 and 8), it is seen that these compounds indeed are burning rate modifiers though not as effective as the previous ones.

The following compound was prepared according to Ralston et al. J. AM. Oil Chemists Soc., 24, page 307:



Mixtures of the above compound with AP (CD-blend) showed final decomposition DTA exotherm at 355°C.

One of the most effective burning-rate depressants reported in the prior art is oxamide. Oxamide was incorporated into

standard propellants at a 1.5 level and compared with the additives of this invention at an 0.3 percent level. The results are shown in FIGS. 9 (Binder No. 2) and 10 (Binder No. 1). For the Binder No. 2 system the quaternary ammonium salt is more than five times as effective as the oxamide. In the Binder No. 1 system, the sulfobetaine shown is even more effective.

The scope of the invention is not limited to amine derivatives; actually any potential base as defined there will be effective although the most powerful burning-rate depressants are derived from amines. An example for this are depressants derived from carboxylic acid salts, preferably from such which are relatively strong acids (e.g., by  $\alpha$ -substitution with electron withdrawing groups):



wherein  $R_1$  = alkyl or aryl (preferably long hydrocarbon chains, e.g.,  $\text{C}_{10}\text{H}_{22}$  and longer);  $R_2$  = preferably  $-\text{OH}$ ;  $R_3=\text{H}$  or aryl and  $Y$  = preferably cations of the alkali or alkaline earth metals, like Li, Na, K, Mg, Ca Sr and Ba.

A example for the preparation of a carboxylic acid salt is Li-benzilate wherein 0.05 moles of benzilic acid\* are dissolved in warm methanol and a solution of 1.2 g. LiOH (in just enough methanol to dissolve it) is added. The Li-salt crystallizes out at room temperature and can be recrystallized from isopropanol. \*(Benzilic acid can be either purchased or made according to "Organic Synthesis" Collective Vol. I, p. 89 (1958), publ. John Wiley & Sons, Inc., New York.

As used herein, potential base means that free bases will not only be released from real chemical compounds, but also from adsorbates, clathrates (inclusion compounds) etc. An example for the latter are amine/urea inclusion compounds, where the amine is contained in channel structures formed by the urea crystal lattice. At the m.p. of the urea (about 130°C.), the amine is released and is free to diffuse through the binder to the  $\text{NH}_4\text{ClO}_4$  particles.

An example for the preparation of an alkylamine urea-clathrate is where 40 g. of urea are dissolved in 100 ml. 10.4 methanol, then 10.4 g. dimethyloctadecylamine are added under stirring; the clathrate crystallizes out on cooling under continued stirring. It is filtered off at room temperature, washed with ice cold methanol and dried under vacuum at room temperature. Titration of the clathrate showed that it contained 75 moles amine per 100 g. clathrate or 22.3 g. amine per 100 g. clathrate.

The present invention is applicable to all types of ammonium perchlorate containing solid propellants including those having polymeric binders derived from polyether-diols, -tris etc., and polybutadiene-diols, -tris etc. with isocyanates as curatives (polyurethanes), or derived from polybutadiene-dicarboxylic acids and aziridines or aziridine derivatives as curatives. The propellants may contain fuels such as aluminum, plasticizers, stabilizers and the like. Many propellant formulations and their processing techniques are disclosed in assignee's prior patents including U.S. Pat. Nos. 3,245,849 and 3,340,111 the disclosure of which are expressly incorporated herein by reference.

Having fully described the invention, it is intended that it be limited only by the lawful scope of the appended claims.

We claim:

1. A novel solid ammonium perchlorate containing rocket propellant composition containing a polymeric organic binder and an effective burning-rate depressing amount of a potential base which is stable under normal solid propellant curing conditions but which upon combustion of the propellant undergoes conversion to form at least some free base, said potential base being an organic nitrogen compound and present in an amount from about 0.01 percent to about 5 percent by weight of the propellant.
2. In solid rocket propellants comprising a cross-linked high molecular weight polymeric binder and an ammonium

perchlorate oxidizing agent, the improvement wherein said propellant contains an effective burning-rate depressing amount of a potential base which is stable under the normal curing conditions for solid rocket propellants but which is capable upon combustion of said propellant of conversion to form at least some free base, said potential base being an organic nitrogen compound and present in an amount from about 0.01 percent to about 5 percent by weight of the propellant.

3. The composition of claim 1 wherein the propellant additionally contains a finely divided metal fuel.

4. The composition of claim 1 wherein the propellant contains a polyurethane binder.

5. The composition of claim 1 wherein the propellant contains a binder comprising a carboxy-terminated polydiolefins cross-linked with aziridines or their derivatives respectively.

6. The composition of claim 1 wherein the potential base is an organic amine precursor.

7. The composition of claim 1 wherein the potential base is

an ammonium salt of an organic amine.

8. The composition of claim 1 wherein the potential base is a quaternary ammonium salt.

9. The composition of claim 1 wherein the potential base is a zwitterionic betaine-type compound.

10. The composition of claim 1 wherein the potential base comprises a substituted organic urea.

11. A method of forming a novel solid rocket propellant comprises forming a castable mixture of a curable polymeric

10 binder, ammonium perchlorate, and a potential base, and thereafter casting the mixture and permitting it to set to form a solid rocket propellant having a depressed burning rate, said potential base being an organic nitrogen compound and present in an amount from about 0.01 percent to about 5 percent by weight of the propellant.

12. The method of claim 11 wherein the potential base is an organic amine precursor.

\* \* \* \* \*